

July 19, 1949.

G. S. EVANS

2,476,590

CATHODE COATING

Original Filed March 14, 1941

Fig. 1.



Fig. 2.



INVENTOR

G. S. EVANS

BY *J.W. Greenhaw*

ATTORNEY

Patented July 19, 1949

2,476,590

# UNITED STATES PATENT OFFICE

2,476,590

## CATHODE COATING

George S. Evans, Fairmont, W. Va., assignor to Westinghouse Electric Corporation, East Pittsburgh, Pa., a corporation of Pennsylvania

Continuation of application Serial No. 383,359, March 14, 1941. This application July 3, 1943, Serial No. 493,338

14 Claims. (Cl. 250—27.5)

1

My invention relates to cathodes for discharge devices and especially to coated cathodes, and the present application is a continuation of my co-pending application, Ser. No. 383,359, filed March 14, 1941.

An object of my invention is to increase the rated peak current per unit area of cathode surface.

Another object is to provide a coated cathode able to withstand overloads without destructive sparking.

Other objects and advantages of the invention will be apparent from the following description and drawing in which:

Fig. 1 is a cross section through a base metal and coating formed thereon according to my invention.

Fig. 2 is a cross section through a base metal and standard coating thereon.

Coated cathodes utilizing alkaline earth oxides are very widely used as cathodes of discharge devices. The peak current demanded of a cathode usually determines its size. The present practice is to rate an oxide coated cathode at around five amperes peak current per square inch of coated area, depending to some extent upon the shape of the cathode. An increase in the capacity of the cathode would naturally be of great advantage.

Unfortunately, alkaline earth oxide cathodes exhibit a phenomenon known as sparking. Sparking is a formation of an arc-like spot on the coated surface when the cathode is overloaded. The arc-like spot moves over the surface, knocking off the coating and soon rendering the cathode inoperable. The bond between the oxide coating and the base metal has a great influence on the ability of the cathode to withstand overloads without sparking, and if a spark spot does form, a good bond will minimize the destruction of the coating resulting from the sparking.

In addition, the cathode voltage drop has great influence on the life of an alkaline earth oxide coating, especially in vapors such as mercury and in the heavy gases. A cathode coating with a lower cathode drop than the present type of coating minimizes the loss of life due to ion bombardment. Furthermore, the manner in which the present alkaline earth oxide coating is applied to the cathode has a great influence on its emission, over-load capacity, and life. A new type of coating which need not be so carefully and exactly applied would be highly desirable.

My invention comprises a new cathode coating

2

which has a higher emission capacity, greater overload capacity, less destruction due to sparking, a lower cathode drop, and requires less skill in applying to its base. I utilize a carbonate of

5 one or more of the alkaline earth metals, and preferably utilize only barium carbonate. The base metal preferably is nickel but may be nickel-cobalt-ferrotitanium sold under the trade name "Konal," or any other suitable metal or alloy.

10 The barium carbonate is preferably ball milled to a small particle size. The barium carbonate is mixed with a binder and then sprayed, painted, or applied by dipping to the base metal as in the prior art. While the cathode may be heat treated according to my invention before mounting it in the tube, I preferably mount the coated cathode in the tube and apply my invention after the tube has been processed during exhaust to the point of cathode activation.

15 20 The invention is to heat the cathode very quickly to a temperature at which the coating fuses. Specifically, the cathode should be heated to around 1100° C. at such a rate that the barium carbonate has small chance to totally or even appreciably decompose due to the heating before 1100° is reached. If the heating of the barium carbonate proceeded slowly as in the present practice of activating the cathodes, then the barium carbonate decomposes to barium oxide and carbon dioxide. The barium oxide will not fuse except at extremely high temperatures.

25 30 The decomposition of the barium carbonate starts at about 500° C. and my invention is to heat the barium carbonate from 500° to a temperature of 1100° C. within thirty seconds, and preferably within twenty seconds or less. This rapid heating provides a phase consisting of barium carbonate with a certain percentage of barium oxide and carbon dioxide in the coating. The barium carbonate-barium oxide phase will fuse to the

35 40 base metal at around 1100° C. and the fluffy granular coating will be transformed into a smooth coating with the evolution of some of the carbon dioxide which has been dissociated from the original coating.

45 50 The fusion of the barium carbonate-barium oxide phase does not seem to be dependent on the alloying of the barium oxide with another metal oxide such as is required in the cathodes known to the art. The rapidly heated barium carbonate will fuse on base metals whose oxides the prior art teaches us will not alloy with barium oxide to produce a satisfactory fused coating. Furthermore, barium carbonate can be fused by quick

heating on platinum, which is a metal that forms so little or no oxide under heating conditions that it is unlikely that fusion will result from platinum oxide and barium oxide.

Tests on cathodes employing my coating indicate that the coating fused on nickel may be rated from twenty to thirty amperes per square inch, depending on the cathode design, as compared to a rating of five amperes per square inch for the standard coating on similar cathodes. The bond between the base metal and the fused coating is so excellent that when a spark spot is formed on the coating due to an overload, only a small point on the coating is affected, as compared to the extensive stripping off of the coating on a standard cathode.

Tests made on standard coating and my fused coating show that the voltage drop for the fused coating, at a certain current up to the current at which sparking occurs, is half the voltage tube drop for the standard coating at the same current. Since the coating fuses, the loose parts of the coating, caused by improper or careless method of application, are melted down to good contact with the base metal or underlying coating.

On the evidence of magnified photographs, I have illustrated in Fig. 1 a cross section through a base metal coated in accordance with my invention, and in Fig. 2 a cross section through a base metal and standard alkaline earth cathode. The standard oxide coated cathode in Fig. 2 shows that the surface has a large specific area and that the coating is continuous. The standard coating is of a semi-ceramic crust in nature, being porous, and having an appreciable thickness. In contrast, a magnification of an oxide surface fused by my method shows in Fig. 1 that the oxide exists in discontinuous patches on the base metal, the base metal being exposed through the discontinuities of the coating. I believe that the discontinuous patches, which contain emission material comparable in quantity to the ordinary coating because the density is greater, produces a more permanent and better bond because the material has fused onto the base metal in such a manner that the coating can better follow the expansion of the base metal due to heating. The ordinary coating, of a crust nature, does not follow the base metal expansion so well, causing the bond to break, with the result that the coating flakes.

A second advantage I believe is obtained with the fused coating as shown by the magnification, is that the high resistance nature of a semi-ceramic crust is obviated by the dense patches. This renders the cathode more resistant to sparking, as tests show. A third advantage I believe is obtained is that the uncovered base metal, which during operation is commonly thought to become active by virtue of barium contamination from adjacent sources of barium, is directly exposed to the discharge path. One theory in the art devised to explain the mechanism of emission from oxide coated cathodes has as its premise emission from the contaminated base metal. In accordance with this theory, the fused coating with exposed emitting base metal areas is believed to give better performance, and tests with my coating confirm this.

In Fig. 1 are disclosed the patches of coating fused to a density of material much higher than that of the standard coating. These discontinuous patches adhere to the base metal and withstand expansion of the base metal. The

appearance of the patches of coating is somewhat globular.

My fused coating has better emission, more indestructibility, lower cathode drop characteristics, and an adherence that lends itself admirably to applications involving high peak currents, such as ignitron firing, spot welding, etc.

I claim:

1. A method of preparing a coated cathode which comprises applying a carbonate of an alkaline earth metal to a base metal and raising the temperature of the coating to approximately 1100° C. before the alkaline earth carbonate is appreciably decomposed due to the heating.

2. The method of preparing a coated cathode which comprises applying a carbonate of barium to a base metal and raising the temperature of the coating to approximately 1100° C. before the barium carbonate is appreciably decomposed due to the heating.

3. The method of preparing a coated cathode which comprises applying an alkaline earth carbonate to a base metal and raising the temperature of the coating from 500° C. to 1100° C. within thirty seconds.

4. The method of preparing a coated cathode which comprises applying an alkaline earth carbonate to a base metal and raising the temperature of the coating from 500° C. to 1100° C. within twenty seconds.

5. The method of preparing a coated cathode which comprises applying barium carbonate to a base metal and raising the temperature of the coating from 500° C. to 1100° C. within thirty seconds.

6. The method of preparing a coated cathode which comprises applying barium carbonate to a base metal and raising the temperature of the coating from 500° C. to 1100° C. within twenty seconds.

7. A thermionic type cathode comprising a substantial base of stable metal thereby capable of withstanding heat and current of the order employed in thermionic cathodes, and a barium oxide barium carbonate compound electron-emitting material on said base in the form of promiscuous discrete particles of irregular size and shape, said material being stable when heated and emissive due to heating the cathode.

8. A cathode comprising a base portion and a fused barium carbonate coating thereon having adhesion to the base portion by fusion therewith and thereon.

9. A cathode comprising a base portion and a fused barium carbonate-barium oxide coating thereon having adhesion to the base portion by fusion therewith and thereon.

10. A cathode comprising a base portion of nickel and a fused barium carbonate coating thereon having adhesion to the base portion by fusion therewith and thereon.

11. A cathode comprising a base portion of nickel and a fused barium carbonate-barium oxide coating thereon having adhesion to the base portion by fusion therewith and thereon.

12. A cathode comprising a base portion of an alloy of nickel-cobalt and ferrotitanium and a fused coating thereon having adhesion to the base portion by fusion therewith and thereon.

13. A cathode comprising a base portion of an alloy of nickel-cobalt and ferrotitanium and a fused barium carbonate coating thereon having adhesion to the base portion by fusion there-

14. A cathode comprising a base portion of an alloy of nickel-cobalt and ferrotitanium and a fused barium carbonate-barium oxide coating thereon having adhesion to the base portion by fusion therewith and thereon.

GEORGE S. EVANS.

**REFERENCES CITED**

The following references are of record in the file of this patent:

**UNITED STATES PATENTS**

| Number    | Name            | Date         |
|-----------|-----------------|--------------|
| 1,813,320 | Schaefer et al. | July 7, 1931 |

| Number       | Name              | Date           |
|--------------|-------------------|----------------|
| 1,905,035    | Marden            | Apr. 25, 1933  |
| 1,909,916    | Duffendack et al. | May 16, 1933   |
| 1,961,122    | Lowry             | May 29, 1934   |
| 5 1,981,245  | Pearcy            | Nov. 20, 1934  |
| 2,015,424    | Forst             | Sept. 24, 1935 |
| 2,065,570    | Essig             | Dec. 29, 1936  |
| 2,075,377    | Varian            | Mar. 30, 1937  |
| 10 2,081,864 | Edwards et al.    | May 25, 1937   |
| 2,172,207    | Kolligs et al.    | Sept. 5, 1939  |
| 2,198,327    | Bandringa et al.  | Apr. 23, 1940  |
| 2,256,341    | Hickok            | Sept. 16, 1941 |